

June 9, 1959

R. R. UNSWORTH

2,890,146

METHOD OF PRODUCING PREFORMED COMBINATION  
UPHOLSTERY AND INSULATOR PADDING

Filed Sept. 21, 1955

2 Sheets-Sheet 1



Fig. 2.



Fig. 1.

INVENTOR  
Raymond R. Unsworth

Morgan, Finnegan, Durham & Pine  
ATTORNEYS

June 9, 1959

R. R. UNSWORTH

2,890,146

**R. R. UNSWORTH**  
**METHOD OF PRODUCING PREFORMED COMBINATION**  
**UPHOLSTERY AND INSULATOR PADDING**

Filed Sept. 21, 1955

2 Sheets-Sheet 2



Fig. 3.



੫  
੮



Fig. 4.

*INVENTOR.*

Raymond R. Unsworth

Morgan, Finnegan, Durham & Pine

*ATTORNEYS*

# United States Patent Office

2,890,146

Patented June 9, 1959

1

2,890,146

## METHOD OF PRODUCING PREFORMED COMBINATION UPHOLSTERY AND INSULATOR PADDING

Raymond R. Unsworth, Burlington, Vt., assignor to Queen City Tuletex Corporation, Burlington, Vt., a corporation of Vermont

Application September 21, 1955, Serial No. 535,565

5 Claims. (Cl. 154—101)

The present invention relates to a novel combination upholstery and insulator padding material for use in mattresses, chairs, furniture and all other cushioning and seatings to be used in conjunction with spring-supporting elements, such as springs of the coil or zigzag type.

The use of upholstery padding in furniture is well known. Very briefly, upholstery padding is that type of padding having an inherent springless or resilience to provide cushioning comfort and the sensation of soft support. Likewise, the use of insulator padding is well known. The function of insulator padding is to insulate or block the feeling of the spring-supporting elements of an article of furniture. Such padding accomplishes the desired blockage by distributing weight over the structure of the spring uniformly to the cushioning (upholstery) padding on the side of use. When properly constructed and utilized, the spring section covered with a proper insulator padding provides uniform support over the whole area of the cushioning, seating or mattress surface. The upholstery padding provides the comfort and softness over this support.

My invention relates to a novel padding having one portion which affords an upholstery or cushioning effect, with the remaining portion providing an insulating effect.

Objects and advantages of the invention will be set forth in part hereinafter and in part will be obvious herefrom, or may be learned by practice with the invention, the same being realized and attained by means of the steps, compositions, combinations and improvements pointed out in the appended claims.

The invention consists in the novel steps, processes, constructions, combinations, and improvements herein shown and described.

An object of my invention is to provide a novel padding which affords cushioning comfort and the sensation of soft support and at the same time functions to block the feeling of spring-supporting elements.

A further object of my invention is to provide a pre-formed, integral combination insulator and upholstery padding which is inexpensive and durable, and which may be produced by the use of conventional apparatus.

Another object of my invention is to provide a pre-fabricated, integral combination pad, preformed to required dimensions, which can be secured to spring-supporting elements of the article to be upholstered by a single simple fastening operation, such as clamping, gluing, hog ringing, sewing, or the like.

Another object of my invention is to provide, through the use of the insulator portion of a combination insulator and upholstery pad, a smooth, firm, consistent surface to which the upholstery fabric may be applied either directly or with a minimum of cotton or cellulose batting.

Another object of my invention is to provide a novel method for producing a padding having the desired qualities stated in the foregoing objects.

I have found that the foregoing objects are realized by the utilization in a novel manner of curled fibrous material of synthetic, animal, vegetable or mineral origin

2

in conjunction with uncurled fibrous material of synthetic, animal, vegetable or mineral origin to form an integral combination upholstery and insulator padding.

More particularly, my novel padding is formed by distributing curled and uncurled fibers separately on a horizontally moving support, such as a moving conveyor belt to build a continuous batt, comprising a layer of curled fibers and a layer of uncurled fibers and applying a bonding agent to bind the fibers together. The bonded batt or composite layer (layer of curled fibers and layer of uncurled fibers) is then pre-dried, sized, dehydrated, cured and cut to the desired dimensions by shearing, slitting, dinking or die-pressing, etc., packed and shipped.

The portion of my novel material comprising the bonded curled fibers provides the desired cushioning comfort and sensation of soft support, while the remaining portion comprising the bonded uncurled fibers affords the desired insulator action.

It should be realized that various modifications may be used in carrying out my invention. For example, the uncurled fibrous material may be deposited onto the conveyor belt before or after the curled material. If the uncurled material is deposited first, the insulator portion is the bottom portion of the initial batt. If the uncurled material is deposited last, the insulator portion is the top portion of the initial batt. The uncurled material is more readily compressible than the curled fibrous material, and, consequently, in sizing the batt for thickness, the straight or uncurled material compresses into a thinner, harder, insulator portion having most of the fibers approximating a single plane, while the curled material is bonded in a resilient spring padding.

Also, the sequence of operations with respect to the bonding of the fibers may be varied. For example, if the uncurled fibers are deposited first on the conveyor belt, the layer of unfurled fibers formed may or may not be sprayed with the bonding agent prior to the addition of curled fibrous material. In like manner, if so desired, the insulator material may be rolled or compressed prior to depositing the curled material on the conveyor. Also, the uncurled material may be interlaced or punched on a needle loom prior to depositing the curled material.

Regardless of the particular method of applying the bonding agent employed, the important thing is that the final layer comprise an integral composite of a layer of uncurled fibrous material bonded together, said layer in turn being bonded to a layer of curled fibrous material bonded together.

Any suitable curled and uncurled fibers may be used in carrying out my invention. Generally, the uncurled fibers forming the insulator portion of my padding are finer and less resilient than the curled fibers forming the upholstery portion of the padding. Examples of typical curled fibers that may be used include such synthetic fibers as monofilaments of polystyrene, vinyl, Saran, nylon, Orlon, rayon, and the like; animal fibers such as horse hair, hog hair, cattle hair; mineral fibers such as steel wool or glass wool; and vegetable fibers such as coir, cocoa, bristle, omat, crin vegetal, Spanish moss, excelsior and the like.

Typical uncurled fibers, which include "sisal tows," henequen, tula, pita, palma and bagasse fibers.

Any suitable vegetable or animal adhesive gum resin or the like, that will bond the uncurled and curled fibers together, may be used. Examples of suitable bonding agents are vulcanizable natural rubber latex, neoprene, G.R.S. and other synthetic or plastic emulsions. Of course, the quantity of bonding agent used will vary depending on the quantity of fibers to be bonded together. Usually, the bonding agent varies in an amount from  $\frac{1}{4}$  to 1 part per part of fibers.

Conventional apparatus, utilized in a novel manner, may be used in carrying out my process. For example,

any traveling surface suitable for receiving a layer of curled and a layer of uncurled fibers may be used, such as the heretofore known conveyors, belts or aprons presently used in forming upholstery paddings. In like manner, any suitable fiber distributing apparatus that will distribute the curled and uncurled fibers to form a composite layer may be used, such as a distributor, a spreader, a lapper of the camel-back type or horizontal type, etc. Also, any suitable means for applying the bonding agent to the layers of curled and uncurled fibers may be used, such as a doctor knife, roll coating, dipping, spraying, etc. Also, any conventional compressing apparatus for compressing the bonded fibers, such as pressure rolls, may be used.

This invention (in a preferred form) is illustrated in the drawings and hereinafter more fully described.

Figure 1 is a top plan view, more or less diagrammatic, of apparatus utilizing three lappers for use in carrying out the continuous method of my invention.

Figure 2 is an elevational view of the device of Figure 1 as seen along either of the lines 2-2 of Figure 1.

Figure 3 is a side elevational view looking towards the spraying and drying section of the apparatus, as indicated by lines 3-3 of Figure 1.

Figure 4 is an enlarged sectional view of the drier section of the apparatus, with parts in elevation.

Figure 5 is a fragmentary perspective view of a fibrous batt made by the method of my invention.

As shown on the drawings:

The reference numerals 10, 10a, 10b, indicate a plurality of feeders, the reference numerals 11, 11a and 11b corresponding garnets, and the reference numerals 12, 12a, 12b corresponding camel-back lappers, each of the foregoing individual pieces of equipment being of conventional design which are known to those in the field in the manufacture of mattress and upholstery bedding.

Each of the feeders 10, 10a, 10b, is provided with corresponding hoppers 13, 13a and 13b. In the particular embodiment shown, fibers 14 are uncurled fibers, and 14a and 14b are curled fibers. It should be understood that the character of the fibers may be varied, depending upon the desired density or type of padding produced.

The fibers 14, 14a and 14b are drawn through a mechanism of their respective feeders 10, 10a and 10b, and automatically measured weights or volumes of the fibers are periodically dropped therefrom onto traveling aprons 15, 15a and 15b, respectively.

In the garnets 11, 11a, 11b, the fibers 14, 14a and 14b, respectively, are picked, or carded, and dropped onto upwardly traveling conveyors 16, 16a and 16b respectively. These conveyors 16, 16a and 16b each constitutes a part of the camel-back lappers 12, 12a and 12b, respectively. Each of the lappers 12, 12a and 12b includes an oscillatable, downwardly-inclined lapper conveyor 17, 17a, 17b. The layers of fibers 18, 18a and 18b which are carried up by conveyors 16, 16a, 16b, respectively, travel downwardly on conveyors 17, 17a and 17b, respectively, and are deposited upon the conveyor 19.

Each of the conveyors 17, 17a and 17b is provided with an oscillatory movement so as to lap the entire width of the conveyor belt. In the particular embodiment shown, as conveyor belt moves forward, curled fibers from conveyor 17b are deposited over the entire width of the conveyor belt to form a layer 20b. As the belt moves forward, additional curled fibers are deposited over the entire layer 20b on conveyor 17a to form a thicker layer 20a of curled fibers. As the belt moves further, uncurled fibers are deposited by conveyor 17 over the entire width from conveyor 17b to form a thicker composite layer 20.

A short, upwardly-inclined conveyor 21 carries the composite layer 20 to spraying apparatus, indicated generally by the reference character S, which may suitably comprise a lower suction chamber 22 and an upper spray head 23. A liquid bonding composition 24 is sprayed onto the moving layer 20 and is drawn by suction through

the batt to thoroughly impregnate and coat the curled fibers thereof. The individual curled fibers are thus uniformly coated with the bonding composition. At the same time, the layer 20 is somewhat compacted by the action of the suction and the liquid bonding composition.

Beyond the spraying apparatus S a conveyor 25 picks up the composite layer 20, and conveys it into drier D. The drier D comprises a chamber, in which are mounted three horizontally disposed conveyors 29, 29a and 29b, superimposed one above the other. A reversing roll 31 is positioned at the delivery end of the drier between the lowermost pass 29 and the intermediate pass 29a. A second reversing roll 32 is positioned at the intake end of the drier between the intermediate pass 29a and the upper pass 29b. Adjustably spaced compressing rolls are arranged in a plurality of sets, such as the set 33 associated with the upper run of the conveyor 29 and set 34 associated with the upper run of the conveyor 29a. Blowers 35 are positioned along the back side of the drier for delivering heated air into the drying chamber.

A second spraying apparatus, indicated generally by the reference character S', may be positioned between the reversing roll 31 and the end of the intermediate conveyor 29a. When passing through the spray apparatus S', the reverse side of the composite layer 20 is sprayed with a bonding composition to thoroughly impregnate and coat the uncurled fibers thereof and part of the curled fibers.

After leaving the spraying apparatus S, the composite web passes over the lowermost conveyor 29, and is subjected to a drying temperature in the neighborhood of 150 to 180° F. After the composite web has been partially dried, it passes between the set of rollers 33, which are spaced to compress the layer into a batt B of approximately the desired thickness. On compression, the layer 20 forms a layer of uniform thickness.

At the spraying apparatus S', the other side of layer 20 is sprayed with a vulcanizable rubber latex so as to insure a uniform coating of the rubber latex over the fiber. It will be understood, however, that if the batt is relatively thin, or if only a light coating of rubber latex is desired, the spray apparatus S' may not be used. Also, while spraying has been found to be most suitable, other means of applying a bonding agent to the fibrous batt may be employed, such as an immersion tank or the like.

During the passage of the laminated web through the drier on the conveyor 29a, it again passes between a set of sizing rolls 34 while in a partially dried condition in order to insure the desired uniform thickness of the finished batt. For some combinations of fibrous materials and bonding agent, only one set of compression rolls located in the sequence at position 34 has proven adequate. In the final pass through the drier, over the uppermost conveyor 29b, the pre-dried composite batt is subjected to sufficiently high temperatures to effect a vulcanization, or cure, of the rubber latex, say in the neighborhood of 225 to 300° F.

The finished batt (Fig. 5) comprises a fibrous layer 40 of loosely associated intermingled fibers, the upper portion 41 of which is uncurled fibers and the lower portion 42 of which is curled fibers, having a coating of a bonding composition, such as vulcanized rubber, over the surfaces thereof, that serves to hold the fibers together. The lower portion 42 possesses a greater resiliency than the upper portion 41 and serves as an upholstery support. The finer, less resilient, uncurled fibers forming upper portion 41 are more readily compressible than the curled fibers forming portion 42; and consequently in sizing the batt for thickness, the uncurled fibers compress into a thinner, harder portion than that formed by the curled fibers to provide an effective insulator portion. Advantageously, the insulator or uncurled fibers may be softened by wetting or steaming or compacting by rollers so as to approximate a single plane. Accordingly, the curled fibers continue to provide a thicker,

fluffier batt possessing a greater amount of resilience than the uncurled portion.

It should be understood that various modifications may be made of the above-described specific embodiment. For example, instead of distributing curled fibers by means of lappers 17b and 17a and uncurled fibers by means of lapper 17, uncurled fibers may be distributed by means of end lappers 17b and 17 and curled fibers by means of middle lapper 17a, resulting in a combination pad comprising a center upholstery portion of curled fibers sandwiched between insulator portions of uncurled fibers. If so desired, in place of the three lappers shown in the preferred embodiment, two lappers may be used, one for distributing curled fibers and one for distributing the uncurled fibers.

My novel method of producing an integral combination upholstery and insulator padding results in a saving in production time, equipment and materials, as compared with the production of an upholstery pad and insulator pad separately. Advantageously, my novel padding may readily be attached to spring-supporting elements of an article of furniture to provide an insulator at its bottom portion and an upholstery portion at its top portion. In short, I have produced a novel combination upholstery and insulator padding for use over spring-supporting elements of furniture which provides an efficient, tough, inexpensive, easy to produce, long-lived, durable and comfortable seating or bedding.

The invention in its broader aspects is not limited to the specific steps, compositions, combinations and improvements described, but departures may be made therefrom within the scope of the accompanying claims without departing from the principles of the invention, and without sacrificing its chief advantages.

What is claimed is:

1. A method for the manufacture of an integral combination insulator and upholstery padding, comprising distributing separately loosely intermingled uncurled fibers and loosely intermingled curled fibers on a generally horizontal traveling surface to provide a layer of 40 uncurled fibers and a layer of curled fibers, applying a

bonding agent to said fibers to bond the fibers together to form an integral final layer.

2. The method of claim 1, wherein the uncurled fibers are finer and less resilient than the curled fibers, and wherein the final layer is compressed for sizing, the uncurled fibers compressing to a higher degree than the curled fibers to provide a stiffer, denser portion than the portion formed by the curled fibers.
3. The method of claim 1, wherein the uncurled fibers are softened so as to approximate a single plane.
4. A method for the manufacture of an integral combination insulator and upholstery padding, comprising distributing loosely intermingled uncurled fibers and loosely intermingled curled fibers in layers on a horizontal surface to provide a layer of uncurled fibers and a layer of curled fibers with an interface of intermingled uncurled and curled fibers, and applying a bonding agent to said fibers to bond the fibers together to form an integral final layer.
5. The method of claim 4, wherein the uncurled fibers are finer and less resilient than the curled fibers, and wherein the final layer is compressed for sizing, the uncurled fibers compressing to a higher degree than the curled fibers to provide a stiffer, denser portion than the portion formed by the curled fibers.

#### References Cited in the file of this patent

#### UNITED STATES PATENTS

|           |                 |       |               |
|-----------|-----------------|-------|---------------|
| 2,341,130 | Unsworth        | ----- | Feb. 8, 1944  |
| 2,385,870 | Lashar et al.   | ----- | Oct. 2, 1945  |
| 2,397,936 | Glidden et al.  | ----- | Apr. 9, 1946  |
| 2,565,941 | Barnard         | ----- | Aug. 28, 1951 |
| 2,571,334 | Browne          | ----- | Oct. 16, 1951 |
| 2,574,849 | Talalay         | ----- | Nov. 13, 1951 |
| 2,580,202 | Talalay et al.  | ----- | Dec. 25, 1951 |
| 2,624,079 | Duvall          | ----- | Jan. 6, 1953  |
| 2,662,044 | Morrison et al. | ----- | Dec. 8, 1953  |
| 2,742,951 | Marc            | ----- | Apr. 24, 1956 |

#### FOREIGN PATENTS

|         |           |       |             |
|---------|-----------|-------|-------------|
| 141,085 | Australia | ----- | May 7, 1951 |
|---------|-----------|-------|-------------|